

[54] METHOD OF TRANSFERRING IMAGES  
PRODUCED BY LIQUID DEVELOPMENT[76] Inventors: **Takashi Saito; Shuniti Kubu**, both  
of Tokyo, Japan; **Canon Kabushiki  
Kaisha**, 03, Tokyo, Japan

[22] Filed: Aug. 30, 1971

[21] Appl. No.: 176,096

## [30] Foreign Application Priority Data

Sept. 4, 1970 Japan..... 45-77872

[52] U.S. Cl. 117/37 LE, 96/1 LY, 96/1.4,

355/10, 117/155 UA

[51] Int. Cl. G03g 13/16

[58] Field of Search 117/37 LE; 96/1 LY, 1.4;  
355/10; 118/637, DIG. 23

## [56] References Cited

## UNITED STATES PATENTS

3,251,688 5/1966 Mihajlov..... 96/1 LY

|           |         |                          |           |
|-----------|---------|--------------------------|-----------|
| 3,419,411 | 12/1968 | Wright .....             | 96/1.4    |
| 3,556,784 | 1/1971  | Robinson et al. ....     | 96/1.4    |
| 3,663,219 | 5/1972  | Takahashi.....           | 117/37 LE |
| T879,009  | 10/1970 | Staudenmayer et al. .... | 117/37 LE |
| T887,027  | 6/1971  | Chechak .....            | 117/37 LE |

Primary Examiner—William D. Martin

Assistant Examiner—M. Sofocleous

Attorney, Agent, or Firm—Fitzpatrick, Cella, Harper  
& Scinto

[57]

## ABSTRACT

In an electrophotographic process, visual images obtained by developing electrostatic latent images with a liquid developer are transferred to a transferring paper having oil absorbing coefficient ranging from  $1.0 \times 10^{-4}$  to  $5.0 \times 10^{-2}$  cm./sec. and smoothness by Bekk tester ranging from 30 to 150 seconds.

4 Claims, 5 Drawing Figures



FIG. 1



FIG. 4



FIG. 2



FIG. 3a



FIG. 3b



## METHOD OF TRANSFERRING IMAGES PRODUCED BY LIQUID DEVELOPMENT

### BACKGROUND OF THE INVENTION

#### 1. Field of the Invention

This invention relates to a method of transferring visual images produced by liquid-developing electrostatic latent images formed on a surface of an electro-photographic photosensitive member.

#### 2. Description of the Prior Art

Heretofore, there have been investigated various transferring methods for images developed by a liquid development. For example, a back side of a transferring paper is earthed by a roller or corona discharging; a bias voltage is applied between a photosensitive member and a transferring paper to enhance the transferring efficiency; or the liquid developer is improved to obtain a good transferring property of a developed image to a transferring paper.

However, there have not been obtained any knowledges of transferring papers used for transferring an image developed by liquid development in electro-photographic processes. When usual papers used for transferring images produced by dry development is used in transferring images produced by liquid development, the transferring efficiency is extremely low and uniform transferred images are not obtained. Furthermore, the liquid developer is absorbed into the transferring paper in a large amount and therefore, it takes disadvantageously much time at the drying and fixing stages. The transferring paper uneconomically takes out much amount of the liquid developer and this results in formation of a large amount of vapor of the carrier liquid in the drying stage and this is not desirable from hygienic point of view.

The transferring of images developed by liquid development in electro-photographic processes is considered to be effected mainly by electrophoresis of toner particles in a liquid (a carrier liquid of a liquid developer) present between a surface of a photosensitive member and a transferring paper. A transferring paper capable of absorbing a large amount of liquid, i.e., a paper of low liquid holdout, decreases an amount of the carrier liquid upon transferring operation and thereby disturbs the electrophoresis of toner particles. As the result, the transferring efficiency is lowered to a great extent and furthermore there occurs non-uniform transferring.

In addition, after transferring, the degree of wetness on the surface of photosensitive member becomes low and this does not favor the cleaning operation.

In transferring images obtained by liquid development, it is necessary to pay attention to a fixing property as well as the above mentioned transferring characteristics of paper.

The inventors have found that transferring papers of low oil absorption property favor the transferring property, but show low fixability for transferred images. This seems due to a fact that toner particles hardly permeates the fibers composing a paper and toner particles can not be fixed to the paper in such a way that the toner particles take root in the fibers. When a surface of paper is coated with a resin so as to prevent permeation of a carrier liquid, the surface property is relatively good, but such treatment lowers the fixability.

Any way, a fixing agent contained in toner can not impart sufficient fixability. However, the present inven-

tors have found that fixability is markedly improved by imparting a certain roughness to a surface of a paper of low oil absorption property. In other words it has been now found that low oil absorption property and rough surface are indispensable conditions for a transferring paper used in transferring of images developed by a liquid developer.

### SUMMARY OF THE INVENTION

According to the process of this invention, there is used a transferring paper having oil absorption coefficient ranging from  $1.00 \times 10^{-4}$  to  $5.0 \times 10^{-2}$  cm./sec., preferred with from  $1.0 \times 10^{-4}$  to  $1.5 \times 10^{-2}$  cm./sec. and smoothness by Bekk tester ranging from 30 to 150 seconds, preferably from 50 to 100 seconds upon transferring an image obtained by developing an electrostatic latent image by a liquid developer to a transferring paper.

When the oil absorption coefficient is higher than  $5.0 \times 10^{-2}$  cm./sec., the transferred image is scratchy and not practical. On the contrary, when the oil absorption coefficient is less than  $1.0 \times 10^{-4}$  cm./sec., the transferring property is good, but there appear many pinholes caused by liquid soaked in the paper and it takes long time to dry. And further the cleaning of the photosensitive member is very difficult after the transferring.

When the smoothness by Bekk tester is higher than 150 seconds, the fixing property is so low that a practical copy can not be obtained. On the contrary, when the smoothness is less than 30 seconds, there appear missing dots.

It is an object of this invention to provide a method of transferring an image obtained by developing an electrostatic latent image formed on a photosensitive member in an electro-photographic process.

It is another object of this invention to provide a method of transferring an image in high efficiency giving a transferred image of high quality.

It is a further object of this invention to provide a transferring method by which there is obtained a good fixation of a transferring paper.

It is still another object of this invention to provide a transferring method in which the cleaning of a photosensitive member surface is very easy after the transferring.

It is still a further object of this invention to provide a transferring method in which the amount of liquid developer absorbed to the transferring paper is small and the drying time can be short and moreover the consumption of liquid developer is low.

### BRIEF DESCRIPTION OF THE DRAWING

FIG. 1 shows schematically a cross section of an apparatus used for a process according to this invention;

FIG. 2 is an enlarged cross section of a part of the apparatus shown in FIG. 1;

FIG. 3 is a graph showing a surface property of a paper measured by a needle touch method; and

FIG. 4 schematically shows an apparatus for measuring oil absorption coefficient.

### DESCRIPTION OF THE PREFERRED EMBODIMENT

A transferring paper used in this invention may be obtained by adjusting the oil absorption coefficient to a range as defined in the claims in the following ways.

1. Incorporating in high ratio a fiber material capable of strengthening beating degree such as cotton material, e.g., rag, hemp, soft wood and the like to make the tissue dense, i.e., lowering permeability.

2. Incorporating a filler such as resin to the tissue or surface, or sizing or coating to lower the permeability.

Measuring method of oil absorption coefficient is illustrated in FIG. 4. One drop of Isopar G 23 (about 0.004 c.c.) is dropped onto a sample paper 27 placed between spacer rings 26 on a support table 28 by using an injector (2 c.c.) 24 having a needle 25 of subcutaneous Lure Type  $\frac{1}{8}$ . The dropped portion is observed from back side of the paper through a mirror 29. A light source is designated as 22.

When Isopar G permeates the sample paper, the corresponding portion of the sample paper becomes transparent. Firstly, the sample becomes partly transparent (pinhole) and then the whole dropped portion (about 10-15 mm in diameter) becomes transparent. There is measured a period of time from a time when a drop of Isopar G reaches the sample paper to a time when the drop liquid permeates throughout the sample portion corresponding to the dropped portion. The measuring is made with 0.1 second unit. One sample paper is measured with respect to 10 different dropped portions and the averaged time is designated as T. The thickness of the sample paper is measured according to JIS-P8118 and is designated as H (cm.).

An oil absorption coefficient,  $\alpha$ , is represented by the formula:

$$\alpha = H/T \text{ (cm./sec.)}$$

where  $\alpha$  is calculated up to significant figure of two digits.

The smoothness of Bekk tester of paper is measured in accordance with JIS-P8119.

Referring to FIG. 3, the two graphs show the surface property of transferring papers measured by a needle touch method. FIG. 3 (a) shows a relatively smooth surface which is of about 500 seconds by Bekk tester and FIG. 3 (b) shows a rough surface which is of about 30 seconds by Bekk tester.

For the same toner, the transferring paper (a) shows an extremely low fixing property while the transferring paper (b) shows a sufficient fixing property. This good fixing property of the rough surface paper appears to be due to the fact that the toner particles are attached to and buried in the lower portion of the uneven surface. The minimum visible point is composed of gathering of several tens of toners having diameter of about 1-10  $\mu$ . Therefore, some of such toners enter the lower portions of the uneven surface and attaches one another as if the toners spreaded deep root in the paper tissue. On the contrary, the toner particles simply cover the surface of the transferring paper in case of (a) above, but there are hardly present entangling between the toner and the paper surface. Usual printing paper has naturally a surface roughness, but the surface

roughness is not generally compatible with low oil absorption property.

The transferring paper used in this invention may be prepared by coating the surface of paper with a resin so as to improve the oil absorptions property of usual printing paper and further by using a paper making wire net of an appropriate mesh (about 65 mesh) upon making the paper or adjusting appropriately the press roller pressure upon calendering so as to lower the oil absorption property and, in addition, make the surface appropriately rough. By using the transferring paper thus prepared, there can be effected uniform transferring in high transferring yield and furthermore the carrier liquid amount permeating a transferring paper is so small that the drying time can be reduced.

As the result, a transferring method in liquid developing process can be realized in which the fixing is excellent and cleaning of the surface of photosensitive member is very easy after transferring due to high transferring efficiency.

FIG. 1 shows schematically an apparatus carrying out transferring of images developed by a liquid developing process. A photosensitive plate 1 has a three-layer structure composed of a conductive base 1a, a photoconductive layer 1b, and an insulating layer 1c. An electrostatic image may be formed on photosensitive plate 1 by a process, for example, that disclosed in Japanese Pat. Publication No. 4223910 or 4324748. That is, the insulating layer 1c is given a uniform charge of one polarity as shown by 2 to bind an electric charge to a portion in photoconductive layer 1b and near the interface between photosensitive layer 1b and insulating layer 1c, and then a D.C. voltage having a polarity opposite to that charged on insulating layer 1c, or AC corona discharge is applied to insulating layer 1c simultaneously with projecting a light image as shown in 3 to form an electrostatic latent image on insulating layer 1c. A blanket irradiation 4 is then applied to release excess charge bound in photoconductive layer 1b to increase the contrast of the electrostatic latent image. The resulting electrostatic latent image is developed by a liquid developer 5 and excess liquid developer is removed by postcharge 9. The developed image is transferred onto a transferring paper 8 by using a transferring roller 6 and then the surface of photosensitive member 1 is cleaned with a cleaning device 7.

Referring to FIG. 2, a developed image as shown in FIG. 1 is transferred to a transferring paper 8 by contacting the transferring paper 8 with the developed image surface by using a transferring conductive roller 14 earthed. A base 1a is also earthed so that a part of positive charge 16 in base 1a induced by negative charge 13 on the surface is divided into the conductive roller 14 and distributed as shown by 17, and most of toners 18 are attracted by the charge 17, moved and transferred to a transferring paper 8 by electrophoresis.

If the oil absorption property of transferring paper 8 is high in such transferring, a thin layer of carrier liquid 5 (e.g., highly insulating liquid such as kerosene, is absorbed to a transferring paper 8 to reduce the amount of the liquid necessary for electrophoresis transferring. As a result, the transferring is effected by a partial electrophoresis transferring and a kind of pressure transferring and thereby only a small amount of the toner is transferred and in addition the image thus transferred is not uniform.

An appropriate amount of liquid developer is necessary upon transferring for the purpose of obtaining high transferring efficiency. Therefore, a transferring paper of low oil absorption is required. Such transferring paper of low oil absorption hardly contains a carrier liquid therein so that drying and fixing are very rapid. For example, cool wind or allowing to stand is sufficient to dry and fix. Therefore, formation of hazardous vapor is so little that employing the low oil absorption paper is advantageous from sanitary point of view. Furthermore, a thin layer of liquid remains on the photosensitive member surface after transferring and this facilitates cleaning.

The transferring method of the present invention is also effective one for a corona bias transferring method in which a transferring paper is laid on a developed image and a corona discharging is applied from the back side since the transferring in corona bias method is also a kind of electrophoresis transferring mechanism.

The following examples are given for illustrating the present invention, but by no means for limiting the present invention.

#### EXAMPLE 1

Electrostatic images were produced on a photosensitive member composed of a conductive support, a photoconductive layer and an insulating layer by using a method as illustrated in FIG. 1 and the resulting electrophotographic images were developed with a liquid developer prepared as shown below

|                                  |       |
|----------------------------------|-------|
| Carbon black                     | 1.5g. |
| Linseed oil-modified alkyd resin | 3g.   |
| Lecithin                         | 40mg. |

The mixture of the above components was ball-milled with 30g. of Solvesso 100 (Trade name) for about 12 hours and then dispersed into 1 liter of Isopar G (Trade name, supplied by Esso) by using a homomixer to produce the liquid developer.

The images developed on the surface of the photosensitive member were subjected to a charge squeezing treatment by a corona charging of -6KV to remove the excess Isopar G.

On the other hand, a paper of high density and surface smoothness of 100 second (Bekk tester) was prepared by forming a fiber composition of three parts of rag contents and seven parts of soft wood contents, strengthening the beating degree, preparing a paper therefrom, applying a machine coat by using a solution of vinyl acetate resin in toluene in an amount of 10 - 15g./m.<sup>2</sup>, and then treating with calender.

The resulting paper had a thickness of 0.047 mm. and an oil absorption coefficient of  $3 \times 10^{-4}$  cm./sec. This paper was used as a transferring paper. It was closely contacted with the developed images after charge squeezing treatment and then peeled off rolling an electroconductive rubber roller which back surface was earthed to produce clear and highly dense transferred images. The fixing property of the transferred image was also very good.

#### EXAMPLE 2

A paper (oil absorption coefficient of about  $7 \times 10^{-2}$  cm./sec.) of mediocre beating degree prepared from eight parts of hard wood contents and two parts of soft

wood contents was coated with an aqueous dispersion of polyvinyl alcohol and clay (solid matter weight ratio, 1:5) in an amount of 2-3g./m<sup>2</sup>. by using a size-press. The resulting coated paper was subjected to a light calender treatment to obtain a transferring paper having an oil absorption coefficient of  $6.0 \times 10^{-3}$  cm./sec. and smoothness of Bekk tester of 60 seconds.

The transferring paper can give a clear, highly dense transferred image of high fixing property when used in an electrophotographic process as shown in Example 1.

#### EXAMPLE 3

The same paper as in Example 2 (oil absorption coefficient, about  $7.0 \times 10^{-2}$  cm./sec.) was coated with an aqueous dispersion of starch and clay (solid matter weight ratio, 1:1) in an amount of 8 g./m<sup>2</sup>. by using a size-press. The resulting paper was calendered to produce a transferring paper having an oil absorption coefficient of  $5.0 \times 10^{-2}$  cm./sec. and smoothness by Bekk tester of 55 seconds.

Then the transferring paper was subjected to an electrophotographic process as described in Example 1 to produce a transferred image of high transferring property and fixability.

#### EXAMPLE 4

The same paper as in Example 2 (oil absorption coefficient, about  $7.0 \times 10^{-2}$  cm./sec.) was coated with an aqueous dispersion of carboxymethyl cellulose and barium sulfate (solid matter weight ratio, 2:1) in an amount of 8 g./m<sup>2</sup>. by using a size-press. The resulting paper was calendered to produce a transferring paper having an oil absorption coefficient of  $3.5 \times 10^{-2}$  cm./sec. and smoothness by Bekk tester of 70 seconds.

Then the transferring paper was subjected to an electrophotographic process as described in Example 1 to produce a transferred image of high transferring property and fixability.

#### EXAMPLE 5

The same paper as in Example 2 (oil absorption coefficient, about  $7.0 \times 10^{-2}$  cm./sec.) was coated with an aqueous dispersion of methylol melamine, cation starch and clay (solid matter weight ratio, 3:2:5) in an amount of 6 g./m<sup>2</sup>. by using a size-press. The resulting paper was calendered to produce a transferring paper having an oil absorption coefficient of  $2.0 \times 10^{-2}$  cm./sec. and smoothness by Bekk tester of 100 seconds.

Then the transferring paper was subjected to an electrophotographic process as described in Example 1 to produce a transferred image of high transferring property and fixability.

#### EXAMPLE 6

The same paper as in Example 2 (oil absorption coefficient, about  $7.0 \times 10^{-2}$  cm./sec.) was coated with an aqueous dispersion of an acrylic resin emulsion, polyvinyl alcohol and titanium dioxide (solid matter weight ratio, 1:1:1) in an amount of 4 g./m<sup>2</sup>. by using a size-press. The resulting paper was calendered to produce a transferring paper having an oil absorption coefficient of  $8.0 \times 10^{-3}$  cm./sec. and smoothness by Bekk tester of 55 seconds.

Then the transferring paper was subjected to an electrophotographic process as described in Example 1 to produce a transferred image of high transferring property and fixability.

#### EXAMPLE 7

The same paper as in Example 2 (oil absorption coefficient, about  $7.0 \times 10^{-2}$  cm./sec.) was coated with an aqueous dispersion of a polyvinylacetate emulsion and sodium alginate (solid matter ratio, 3:2) in an amount of 3 g./m<sup>2</sup>, by using a size-press. The resulting paper was calendered to produce a transferring paper having an oil absorption coefficient of  $1.0 \times 10^{-3}$  cm./sec. and smoothness of Bekk tester of 120 seconds.

Then the transferring paper was subjected to an electrophotographic process as described in Example 1 to produce a transferred image of high transferring property and fixability.

#### EXAMPLE 8

The same paper as in Example 2 (oil absorption coefficient, about  $7.0 \times 10^{-2}$  cm./sec.) was coated with an aqueous dispersion of NBR latex, casein and clay (solid matter weight ratio, 1:1:2) in an amount of 5 g./m<sup>2</sup> by using a size-press. The resulting paper was calendered to produce a transferring paper having an oil absorption coefficient of  $1.5 \times 10^{-2}$  cm./sec. and smoothness by Bekk tester of 35 seconds. Then the transferring paper was subjected to an electrophotographic process as described in Example 1 to produce a transferred image of high transferring property and fixability.

#### EXAMPLE 9

The same paper as in Example 2 (oil absorption coefficient, about  $7.0 \times 10^{-2}$  cm./sec.) was coated with an aqueous dispersion of an acryl-vinylacetate copolymer emulsion, starch and titanium dioxide (solid matter weight ratio, 2:1:1) in an amount of 5 g./m<sup>2</sup>, by using a size-press. The resulting paper was calendered to produce a transferring paper having an oil absorption coefficient of  $9.0 \times 10^{-4}$  cm./sec. and smoothness by Bekk tester of 65 seconds.

Then the transferring paper was subjected to an electrophotographic process as described in Example 1 to produce a transferred image of high transferring property and fixability.

#### EXAMPLE 10

An ordinary grade paper (oil absorption coefficient,  $2.0 \times 10^{-1}$  cm./sec.) was machine-coated with an aqueous dispersion of an acrylic acid ester and titanium dioxide (solid matter weight ratio, 1:1) in an amount of 8 g./m<sup>2</sup>, and then calendered lightly to obtain a transferring paper having an oil absorption coefficient of  $4.5 \times 10^{-3}$  cm./sec. and smoothness by Bekk tester of 90 seconds.

Then the transferring paper was subjected to an electrophotographic process as described in Example 1 to produce a transferred image of high transferring property and fixability.

#### EXAMPLE 11

An ordinary grade paper was machine-coated with an aqueous dispersion of high styrene latex and NBR latex (solid matter weight ratio, 1:1) in an amount of 10 g./m<sup>2</sup>, and then calendered lightly to obtain a transferring paper having an oil absorption coefficient of  $5.0 \times$

$10^{-3}$  cm./sec. and smoothness by Bekk tester of 100 seconds.

Then the transferring paper was subjected to an electrophotographic process as described in Example 1 to produce a transferred image of high transferring property and fixability.

#### EXAMPLE 12

An ordinary grade paper was machine-coated with an aqueous dispersion of a polyvinyl acetate emulsion, polyvinyl alcohol and barium sulfate (solid matter weight ratio, 1:1:2) in an amount of 15-20 g./m<sup>2</sup>, and then calendered lightly to obtain a transferring paper having an oil absorption coefficient of  $1.0 \times 10^{-4}$  cm./sec. and smoothness by Bekk tester of 150 seconds.

Then the transferring paper was subjected to an electrophotographic process as described in Example 1 to produce a transferred image of high transferring property and fixability.

#### EXAMPLE 13

An ordinary grade paper was machine-coated with an aqueous dispersion of acrylic acid ester and starch (solid matter weight ratio, 1:1) in an amount of 10 g./m<sup>2</sup>, and then calendered lightly to obtain a transferring paper having an oil absorption coefficient of  $8.0 \times 10^{-3}$  cm./sec. and smoothness by Bekk tester of 75 seconds.

Then the transferring paper was subjected to an electrophotographic process as described in Example 1 to produce a transferred image of high transferring property and fixability.

#### EXAMPLE 14

An ordinary grade paper was machine-coated with an aqueous dispersion of NBR latex, methyl cellulose and clay (solid matter weight ratio, 2:3:5) in an amount of 10 g./m<sup>2</sup>, and then calendered lightly to obtain a transferring paper having an oil absorption coefficient of  $7.5 \times 10^{-4}$  cm./sec. and smoothness by Bekk tester of 120 seconds.

Then the transferring paper was subjected to an electrophotographic process as described in Example 1 to produce a transferred image of high transferring property and fixability.

#### EXAMPLE 15

An ordinary grade paper was machine-coated with an aqueous dispersion of a vinyl acetate-styrene copolymer emulsion and barium sulfate (solid matter weight ratio, 1:3) in an amount of 10 g./m<sup>2</sup>, and then calendered lightly to obtain a transferring paper having an oil absorption coefficient of  $7.0 \times 10^{-3}$  cm./sec. and smoothness by Bekk tester of 110 seconds.

Then the transferring paper was subjected to an electrophotographic process as described in Example 1 to produce a transferred image of high transferring property and fixability.

#### EXAMPLE 16

An ordinary grade paper was machine-coated with a solution of acrylic acid ester in toluene in an amount of 30 g./m<sup>2</sup>, lightly calendered and matted by a sand blast method to obtain a transferring paper having unevenness of average  $20\mu$  on the surface, oil absorption coef-

ficient of  $5.0 \times 10^{-3}$  cm./sec. and smoothness by Bekk tester of 45 seconds.

Then the transferring paper was subjected to an electrophotographic process as described in Example 1 to produce a clear transferred image of high transferring property and fixability.

The following Table 1 is given for summarizing the results in the above mentioned examples and comparing them with control shown in Comparison Examples below.

Table 1

| Transferring Method       | Density of Transferred Image         | Density of Image after Fixing Test | Oil Absorption Coefficient of Transferring Paper | Smoothness by Bekk Tester |
|---------------------------|--------------------------------------|------------------------------------|--------------------------------------------------|---------------------------|
| <b>Example</b>            |                                      |                                    |                                                  |                           |
| 1                         | 1.50                                 | 1.41                               | $3.0 \times 10^{-4}$                             | 100                       |
| 2                         | 1.45                                 | 1.40                               | $6.0 \times 10^{-3}$                             | 60                        |
| 3                         | 1.38                                 | 1.34                               | $5.0 \times 10^{-2}$                             | 55                        |
| 4                         | 1.26                                 | 1.24                               | $3.5 \times 10^{-2}$                             | 70                        |
| 5                         | 1.12                                 | 1.04                               | $2.0 \times 10^{-2}$                             | 100                       |
| 6                         | 1.40                                 | 1.38                               | $8.0 \times 10^{-3}$                             | 55                        |
| 7                         | 1.37                                 | 1.29                               | $1.0 \times 10^{-3}$                             | 120                       |
| 8                         | 1.20                                 | 1.19                               | $1.5 \times 10^{-2}$                             | 35                        |
| 9                         | 1.56                                 | 1.48                               | $9.0 \times 10^{-4}$                             | 65                        |
| 10                        | 1.45                                 | 1.37                               | $4.5 \times 10^{-3}$                             | 90                        |
| 11                        | 1.42                                 | 1.35                               | $5.0 \times 10^{-3}$                             | 100                       |
| 12                        | 1.50                                 | 1.40                               | $1.0 \times 10^{-4}$                             | 150                       |
| 13                        | 1.35                                 | 1.32                               | $8.0 \times 10^{-3}$                             | 75                        |
| 14                        | 1.42                                 | 1.35                               | $7.5 \times 10^{-4}$                             | 120                       |
| 15                        | 1.38                                 | 1.31                               | $7.0 \times 10^{-3}$                             | 110                       |
| 16                        | 1.51                                 | 1.50                               | $5.0 \times 10^{-3}$                             | 45                        |
| <b>Comparison Example</b> |                                      |                                    |                                                  |                           |
| 1                         | 0.98                                 | 0.95                               | $7.0 \times 10^{-2}$                             | 40                        |
| 2                         | 1.58<br>(Many Pinholes in the Image) | 1.21                               | $6.0 \times 10^{-5}$                             | 400                       |
| 3                         | 1.25<br>(Remarkable Missing dots)    | 1.22                               | $5.0 \times 10^{-3}$                             | 25                        |
| 4                         | 1.07                                 | 0.98                               | $4.0 \times 10^{-2}$                             | 200                       |

(Density of image was measured by a reflecting densitometer. The density of image before transferring was constantly 1.70.)

### COMPARISON EXAMPLE 1

As the transferring paper, there was used a paper composed of eight parts of hard wood and two parts of soft wood, mediocre beating degree, oil absorption coefficient of  $7.0 \times 10^{-2}$  cm./sec., and surface smoothness by Bekk tester of 40 seconds and an electrophotographic process was carried out in a way similar to Example 1.

### COMPARISON EXAMPLE 2

An ordinary grade paper was machine-coated with an aqueous dispersion of a polyvinyl chloride emulsion, polyvinyl alcohol and barium sulfate (solid matter weight ratio, 1:1:2) in an amount of 30g./m<sup>2</sup>. and calendered to produce a paper having oil absorption coefficient of  $6.0 \times 10^{-5}$  cm./sec., and smoothness by Bekk tester of 400 seconds. The resulting paper was used as a transferring paper and an electrophotographic process was carried out in a way similar to Example 1.

### COMPARISON EXAMPLE 3

An ordinary grade paper was machine coated with an aqueous dispersion of a polyvinyl acetate emulsion, polyvinyl alcohol, and barium sulfate (solid matter weight ratio, 1:1:2) in an amount of 20g./m<sup>2</sup>, calen-

dered and matted by a sand blast method to obtain a paper having oil absorption coefficient of  $5.0 \times 10^{-3}$  and smoothness by Bekk tester of 25 seconds. The resulting paper was used as transferring paper to effect an electrophotographic process in a way similar to Example 1.

### COMPARISON EXAMPLE 4

A paper composed of eight parts of hard wood and 10 two parts of soft wood and having a mediocre beating

40 degree was strongly calendered to produce a paper having oil absorption coefficient of  $4.0 \times 10^{-2}$  cm./sec., and smoothness by Bekk tester of 200 seconds. The resulting paper was used as a transferring paper in an electrophotographic process similar to that of Example 1.

45 The fixing test was carried out as follows. A transferring paper after image-transferred and dried was placed on a horizontal surface plate and a soft paper having a rough surface, "Kojin Wiper" (trade name, supplied by Kojin) of about 8 cm<sup>2</sup> was placed thereon and further an aluminum block was placed on the soft paper of rough surface. The resulting total load was about 12g./cm<sup>2</sup>. The soft paper of rough surface and the aluminum block were fixed in such a way that they can not move to the horizontal direction and then the transferring paper was pulled at a speed of about 7 cm./sec. and this pulling was repreated five times.

50 It is clear from the results as shown above that a paper having oil absorption coefficient ranging from  $1.0 \times 10^{-4}$  to  $5.0 \times 10^{-2}$  cm./sec., particularly from  $1.0 \times 10^{-4}$  to  $1.5 \times 10^{-2}$  cm./sec., is of high transferring property and further a paper having smoothness by Bekk tester of 30 - 150 seconds, particularly, 50 - 100 seconds, shows good fixing property.

11

A paper having oil absorption coefficient higher than  $5.0 \times 10^{-2}$  cm./sec. (of. Comparison Example 1) shows an extremely bad transferring property. On the contrary, when the oil absorption coefficient is less than  $1.0 \times 10^{-4}$  cm./sec., there disadvantageously appear many pinholes in the transferred image.

When the smoothness by Bekk tester is higher than 150 seconds, the fixing property is lower. When the smoothness by Bekk tester is less than 30 seconds, the surface of paper is uneven and many missing dots appear.

We claim:

1. A method of transferring an image developed by a liquid developer which comprises developing an electrostatic latent image formed on a surface of a photosensitive member by an electrophotographic process by using a liquid developer for electrophotography composed of charged fine toner dispersed in a highly insulating liquid and transferring by electrophoresis the de-

12

veloped image to a transferring paper having an oil absorption coefficient from about  $1.0 \times 10^{-4}$  to  $5.0 \times 10^{-2}$  cm./sec. and smoothness by Bekk tester from about 30 to 150 seconds, in the presence of the highly insulating liquid on a surface of the photosensitive member.

2. A method of transferring an image according to claim 1 wherein the oil absorption coefficient is from about  $1.0 \times 10^{-4}$  to  $1.5 \times 10^{-2}$  cm./sec. and the smoothness by Bekk tester from about 50 to 100 seconds.

3. A method of transferring an image according to claim 1 wherein the photosensitive member is a three-layered photosensitive member composed of a conductive support, a photoconductive layer and an insulating layer laminated according to the above-mentioned order.

4. A method of transferring an image according to claim 3 wherein the transferring paper contains a resin.

\* \* \* \* \*

20

25

30

35

40

45

50

55

60

65